

Dec. 2, 1924.

1,517,354

H. W. GILLETT

PROCESS FOR IMPROVING METALS AND ALLOYS IN RESISTANCE TO REPEATED STRESS

Filed April 10, 1923



10,000 50,000 500,000 5,000,000 50,000,000  
Number of Alternations of Stress. Logarithmic Scaling.

Inventor:  
Horace W. Gillett

Patented Dec. 2, 1924.

1,517,354

# UNITED STATES PATENT OFFICE.

HORACE W. GILLETT, OF ITHACA, NEW YORK.

## PROCESS FOR IMPROVING METALS AND ALLOYS IN RESISTANCE TO REPEATED STRESS.

Application filed April 10, 1923. Serial No. 631,191.

(FILED UNDER THE ACT OF MARCH 3, 1883, 22 STAT. L., 625.)

*To all whom it may concern:*

Be it known that I, HORACE W. GILLETT, a citizen of the United States, residing in Ithaca, in the county of Tompkins and 5 State of New York, have invented a new and useful Process for Improving Metals and Alloys in Resistance to Repeated Stress, of which the following is a specification.

This application is made under the act of 10 March 3, 1883, C. 143, (U. S. Stat., 22, p. 625).

One object of my invention is to alter the properties of a metal or alloy so that it will withstand repeated stress or cyclic variations of stress for a longer period than such cyclic stress can be resisted by unaltered metals and alloys.

Another object is to increase the range of cyclic stress which a metal or alloy can 20 withstand without failure.

A further object is to increase the resistance of metals and alloys to repeated stress to an extent greater than, and superimposed upon, the known increase in such resistance 25 that can be obtained by such an operation as forging, rolling, drawing, spinning, etc., or by heat-treatment, or both.

If different specimens of a given metal or alloy be subjected to cyclic variations of 30 stress, as in repeated bending, in rotary bending of a loaded bar, or in reversed axial stress, i. e., in repeated tension and compression, it is found that as the stress range to which the material is subjected is decreased 35 the number of alternations of stress which the specimen will withstand before cracking or breaking increases. If the stress or stress range be plotted against the number of cycles, a curve of the general type of Fig. 1 40 (in which stress is plotted on an ordinary scale, and number of alternations on a logarithmic scale) is obtained in which, at some particular stress or stress range as at A, the relation between stress or stress range and life changes. At stresses above A the life increases slowly with decrease in stress, while at those below A, the life increases 45 rapidly with decrease in stress.

The stress corresponding to the point A, 50 the curvature or slope of the curve at stresses above and below that corresponding to A, and the number of cycles corresponding to the point A, may be different in different metals and alloys, in different states

of hardness, internal structure, purity, cleanliness, etc.

The stress corresponding to the point A may, in some metals or alloys be above the static elastic limit or the static yield point 55 of the material when tested without cyclic stressing, and in other metals or alloys, it may be below.

The stress corresponding to point A may be considered as a cyclic elastic limit or an endurance limit, as it is commonly termed. It is also called the "safe range" of stress, and it is sometimes considered that at lower stress ranges than the safe range failure will never ensue. But as no tests can be made 65 over an infinite period of time it is impossible to establish experimentally whether or not there is a range of stress at which failure will never occur. For engineering purposes, however, it is of value to know at 70 what stress range the relation between stress and life changes, and the endurance limit is the stress at which this relation changes. In the actual case of a quenched and tempered alloy steel with a Brinell hardness of 75 about 400 in a reversed bending test, the point A is at about 100,000 lbs. per sq. in. stress in tension and compression, or a stress range of 200,000 lbs. per sq. in., and at about 750,000 alternations, under the conditions of 80 the test.

If a bar of this material is stressed to 116,000 lbs. per sq. in. it will break in about 100,000 alternations, and one stressed to 110,000 lbs. per sq. in., in about 140,000 85 alternations.

If, however, instead of initially stressing the bar above the endurance limit of about 100,000 lbs. per sq. in. it is initially stressed at a stress below the endurance limit but 90 near to it, in the actual case, at 97,000 to 99,000 lbs. per sq. in., for a considerable number of alternations, in the actual case 1,400,000 to 1,500,000, an improvement in the bar takes place by which the bar is 95 strengthened. If the stress is then raised, the strengthened bar does not break in as few alternations as an un-strengthened bar does. If, after a period of stressing at the new stress the stress is again increased, further strengthening takes place. The increase of stress can take place in steps or it may be gradually and progressively increased.

In the actual case, shown in Fig. 1, a bar (B') first stressed for 1,500,000 alternations at 97,000 lbs. per sq. in. was then stressed at 101,000 lbs. per sq. in. (see point B'') for 5 1,100,000 alternations, and then when tested at 110,000 lbs. per sq. in. (see point B'''), it broke at 650,000 alternations, although an un-strengthened bar (B) breaks at 140,000 alternations at that stress. The life at 10 110,000 lbs. per sq. in. has thus been increased over 4½ times by the strengthening process.

Another bar (C') first stressed at 99,000 lbs. per sq. in. for 1,400,000 alternations, 15 then at 104,000 lbs. per sq. in. (see point C'') for 1,250,000 alternations, then at 111,000 lbs. per sq. in. (see point C''') for 1,350,000 alternations and then tested at 116,000 lbs. per sq. in. (see point C''''), 20 broke after 1,800,000 alternations, although an un-strengthened bar C breaks after 95,000 alternations at that stress. The life at 116,000 lbs. per sq. in. has thus been increased about 190 times by the strengthening process. In Fig. 1 the points showing the stresses and alternations of the bars referred to above are plotted with circles and arrows where the bars did not break and with crosses where they did break.

25 Although a hard heat-treated alloy steel has been chosen as an example, the strengthening process applies to iron and soft steels and to non-ferrous metals and alloys as well.

I am aware that it has been suggested that 30 the properties of metals and alloys may be improved through raising the yield point by overstressing, i. e. stressing above the yield point or elastic limit either in tension or compression, after which overstress the material may behave elastically up to the stress so impressed, and that this may either be done at elevated temperatures or the temperature may be thereafter raised for tempering or annealing purposes. But such overstress, producing permanent set in the material, is attended by a decrease in the elastic limit in compression if the applied over-stress is a tension stress, or a decrease in the elastic limit in tension of the applied over-stress is a compressive stress. That is, by overstressing above the elastic limit the material may be materially improved against either tensile or compressive stress, but not against both.

My process for improvement by under-stressing below the endurance limit is sharply differentiated from the above-mentioned processes, because the under-stressing process improved the material against both tensile and compressive stresses, as is shown by the results plotted in Fig. 1, in which the test specimens were all subjected to equal alternating tensile and compressive stresses in reversed bending.

It is further differentiated in that instead

of a single or a very few applications of stress, my process involves the repetition of the stress below the endurance limit many times.

Still further differentiation is found in 70 the fact that in the overstressing process no improvement is shown in metals or alloys unless the stress is so great as to cause a detectable permanent set in the material, while the process of repeated under-stressing 75 will generally, and in such materials as most commercial steels always, produce no detectable permanent set whatever. My process involves no change in the external dimensions of the material operated upon in cases 80 when the endurance limit is below the elastic limit, which is usual.

The under-stressing process is so called because it must start by stressing below the endurance limit. After the material has 85 been strengthened and its endurance limit raised above its initial value, the process can be hastened by raising the stress, but still keeping it below the now increased new endurance limit. The stress may be increased in steps, or it may be steadily increased, or increased at varying rate. An automatic increase of stress may accordingly be arranged for in the apparatus by 90 which the stress is applied so that as the endurance limit rises the applied stress rises, following the endurance limit but keeping below it. When the stress is steadily increased, it might, for example, be increased 95 at the rate of a tenth of a pound per square 100 inch per cycle of stress, while, when it is increased at a varying rate it might be increased first at say one tenth of a pound per square inch and later at two tenths of a pound per square inch per cycle. 105

The strengthening process may be carried out at elevated temperatures since the interval change or readjustment which results in strengthening appears to be accelerated by increase in temperature. Of 110 course in the case of a metal or alloy whose initial properties have been obtained by cold rolling or a similar strain-hardening process or by quenching and tempering, too high a temperature would soften the material by 115 annealing or tempering, so that there will be an upper limit of temperature for the strengthening process which will vary with the particular material in question. The process could also be carried out at lowered 120 temperatures, although this will usually be a disadvantage rather than an advantage.

The strengthening process may be applied to a finished part of a machine, for example, by running the machine first at light loads 125 and later increasing the load. This is common practice, and while the usual reason for it is to wear in the bearings, it may readily bring about some of the strengthening process, even though the operator of 130

the machine does not know that strengthening takes place.

It is, however, a new procedure in the preparation for use of metals and alloys to 5 intentionally subject them before final assembly and initial use in the finished machine to a strengthening process of repeated stressing with the object of increasing their ability to withstand repeated stress.

10 The strengthening process can be applied to a finished part by loading it in a similar manner to that in which it will be loaded in use. It can be applied to a partly finished part or to unfinished material. For example, an axle shaft could be rotated in an apparatus similar to the well known "Farmer-type" of rotary bending endurance testing machine. A finished connecting rod for a gas engine could be put in repeated tension and compression, or, the rough forging could be similarly stressed and later finished to size. Or, a block of metal could be so stressed, strengthened throughout, and any piece desired can be later machined therefrom. Other applications of my invention 25 to other cases are self-evident.

I do not limit myself to any particular apparatus or method of producing repeated stress, to any specific metals or alloys, to 30 any specific temperature of operation, nor to any particular combination of applied repeated stresses. The applied repeated stress may vary from zero or from a finite tensile or compression stress, for example, 35 to another finite tensile or compression stress. The important limitation is that the initial stress or stress range which is to be repeated be below the endurance limit (respectively stress or stress range) of the particular material for that sort of stress. The initial stress may be close to or well below the endurance limit, but in practice, it will naturally be not very far below it. One 40 advantage of using an initial stress near the endurance limit and of repeating that stress for a considerable number of alternations is that a defective piece, containing surface imperfections or internal flaws of any nature which tend to increase the local stress at any point as distinguished 45 from the stress calculated from the load applied and the dimensions of the piece, will fail under the initial repeated stressing so that the process will tend to seek out and 50 eliminate such defective pieces as well as to strengthen pieces that are not notably defective.

I do not limit myself to any particular steps of increase in stress, to any particular 55 rate of increase of stress with a number of alternations, nor any particular speed of

alternations of stress, since these will vary with the material, with the result desired and with the apparatus used to bring about the strengthening process.

65

Nor do I limit myself by any particular theoretical explanation of the exact phenomena occurring in the strengthening process, since the process is an experimentally observed fact for which different explanations may be adduced.

70

I am aware that other investigators have observed a similar strengthening of materials in the course of endurance tests and I do not claim the process as a method of 75 testing.

80

I do broadly claim the application of the strengthening process as a step in the industrial preparation of materials to withstand repeated stress.

What I claim as new and wish to protect by Letters Patent is:

1. The process of strengthening metals or alloys in their endurance against repeated stress by subjecting them to repeated stress 85 of magnitude not greater than the stress corresponding to the endurance limit of the material.

2. The process of claim 1 followed by further subjection to repeated stress at one 90 or more stresses above the original endurance limit of the material which it had before undergoing the process of claim 1.

3. The process of claim 2 carried out at stresses increased at a constant rate. 95

4. The process of claim 2 carried out at stresses increased at a varying rate.

5. The process of claim 2 carried out at stresses increased partly at a constant rate and partly at a varying rate. 100

6. The acceleration of the strengthening process of claim 1 by carrying out the process at a temperature above room temperature.

7. The acceleration of the strengthening 105 process of claim 2 by carrying out the process at a temperature above room temperature.

8. The acceleration of the strengthening process of claim 3 by carrying out the process 110 at a temperature above room temperature.

9. The acceleration of the strengthening process of claim 4 by carrying out the process at a temperature above room tempera- 115 ture.

10. The acceleration of the strengthening process of claim 5 by carrying out the process at a temperature above room tempera- ture.

HORACE W. GILLETT.